

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL AND METHOD OF MAKING SAME

No Drawing.

Application filed December 21, 1925. Serial No. 76,905.

In the art it has been the practice to use ordinary asphaltic or bituminous materials in the preparation of expansion joints, and in many of these cases, finely divided, saturated, fibrous material. Asphalts of various kinds, except at a very low melting point and very high penetration, at 32° F. become very brittle in winter, and the shock often breaks this material leaving the joint in a manner to 10 destroy its efficiency.

The primary object of this invention is to overcome the brittleness of ordinary asphaltic or bituminous materials and convert them into a normally non-brittle, plastic and elastic 15 material.

Briefly, this invention relates to a treatment of the bituminous material with a glutinous agent or mixture, in order to add to the life of the asphalt or bituminous material and at 20 the same time make the material more elastic.

This glutinous agent or mixture may be prepared by mixing ordinary flour gluten with water, adding glycerine and heating to between 200 and 300 degrees F., creating a 25 viscous, sticky mass. The amount of water required for this purpose will depend on the physical condition of the gluten. Anyone practising the invention and knowing it is desirable to reduce the gluten to a jelly-like, 30 colloidal form will know when to stop adding water. Sufficient glycerine will be added to prevent the watered gluten from hardening. With the water and glycerine added to the 35 gluten it is subjected to a temperature between 200 and 300 degrees F., so as to amalgamate the glycerine with the gluten. During this heat treatment much of the water will be evaporated, but it will not affect the resultant mixture. Should it be found that too 40 much of the water is lost more will be used, in the first place to compensate for any loss of moisture during the heating operation. After a thorough amalgamation has been accomplished with the gluten and glycerine it 45 may be mixed with the asphalt. This step may be conveniently accomplished by utilizing mechanical mixing apparatus in which the melted asphalt is poured, and with the mixer equipped with a steam jacket, or other heating means, so as to keep the materials heated

during mixing. The gluten glycerine compound is added to the mechanical mixer and thoroughly mixed with the asphalt. Proportions may be varying proportions, ranging from five (5) per cent upward of the glutinous 55 solution and ninety-five (95) per cent downward of the asphaltic material.

Another effect upon this bituminous material would be to control its penetrating power, reducing it to a minimum, thus making it 60 easy to incorporate cellular, fibrous material, such as, cocoanut fibre, sisal, flat fibrous vegetable matter, bristles, flax, bagasse, straw, or any other material suitable as a binder, which is to be incorporated and mixed in a manner 65 so that the bituminous material will not penetrate the fibre.

This combination of materials may be effected by the glutinous mixture described, employing varying proportions of the glutinous material, one formula being about five (5) per cent glutinous material and about ninety-five (95) per cent of suitable bituminous material, or varying proportions, increasing the proportion of glutinous material 70 and decreasing the proportion of bituminous material, depending upon the consistency of the mass desired. Where it is desirable to incorporate any of the fibrous material mentioned, percentages varying from three to 80 twenty-five per cent may be readily incorporated with mechanical mixers, known to the art.

I do not wish to be limited to the fibrous matter mentioned, as many other types of 85 fibrous matter may be suitable. Also finely divided matter may be employed, if it is desirable that the entire mass be waterproofed. The resulting product is one of an elastic nature and one which will prolong the life 90 of the asphalt or bituminous material, and at the same time strengthen the binding material resulting from the mixture.

After mixing this material, as outlined, in any suitable mechanical mixer, it may be presented to pressing rolls, also previously known to the art, suitable for reducing the batch to flat sheets, then cutting said sheets into strips, adapting the material for use as premoulded 95 expansion joints.

## I claim:

1. An expansion joint of the class described, comprising a ductile bituminous material having a small quantity of adhesive agent incorporated therewith, said agent having the properties of prolonging the stickiness of the bituminous material and adding elasticity thereto.
2. An expansion joint of the class described, comprising a ductile bituminous material combined with a small quantity of glutinous mixture and having a fibrous material incorporated therewith.
3. An expansion joint of the class described, comprising a ductile bituminous material combined with a subordinate proportion of glutinous mixture and having a finely divided fibrous material incorporated therewith.
4. An expansion joint of the class described, comprising a ductile bituminous material combined with a subordinate proportion of glutinous mixture and having vegetable fibres of varying dimensions, and in an unpenetrated state, incorporated therewith.
5. Preformed construction material, consisting of a mixture of about five (5) per cent gluten, about eighty-five (85) per cent ductile bituminous material and about ten (10) per cent finely divided filling material.
6. The method of preparing a premoulded expansion joint by mixing a gluten, bituminous filling material into a homogeneous mass and finely divided material, reducing same to flat sheets and cutting said sheets into strips of desired size.
7. The method of preparing constructional material by adding gluten to bituminous material for controlling the penetrating powers of the bituminous material, then incorporating fibrous material after said penetration has been controlled, thus minimizing penetration of the fibrous material by the bituminous material.
8. Preformed constructional material consisting of a mixture having a predominating proportion of ductile bituminous material and a subordinate proportion of glutinative agent.
9. The method of preparing constructional material which consists in mixing ordinary flour gluten with water, adding glycerine and heating to a temperature between 200° and 300° F., and adding bituminous material thereto.
10. The method of forming constructional material which consists in mixing flour gluten with water, adding glycerine and heating the same to between 200° and 300° F., and then adding a large proportion of bituminous material thereto.
11. The method of preparing constructional material which consists in mixing flour gluten with water to reduce it to substantially a colloid form, adding sufficient

glycerine to prevent the watered gluten from hardening, heating the mixture to a temperature between 200° and 300° F. and then mixing in a large proportion of bituminous material and heating the mixture during mixing. 70

Signed at Chicago, Illinois, this 16 day of December, 1925.

ALBERT C. FISCHER.